

Patented Oct. 9, 1928.

1,687,454

# UNITED STATES PATENT OFFICE.

CARL ADOLPHE KLEIN, OF BRIMSDOWN, AND ROBERT SKIRVING BROWN, OF LONDON, ENGLAND.

## GLASS, SAND, OR FLINT PAPER, EMERY CLOTH, OR LIKE ABRASIVE.

No Drawing. Application filed October 28, 1925, Serial No. 65,487, and in Great Britain August 26, 1925.

This invention relates to that class of glass, sand or flint paper, emery cloth or like abrasive, which is waterproof so that it can be used on damp or wet surfaces without being 5 affected by the moisture.

Various attempts have been made to prepare abrasive paper or other material of this class, but in all instances these prior processes involve in some way the use of a lead or similarly poisonous dryer, thus nullifying one of 10 the most important properties of such waterproof papers, more particularly when used dry.

Now it has been found that by the use of 15 the process described in the specification of our application for patent, Serial No. 65,486 of even date herewith a waterproof sand paper (or like abrasive) is obtained in which no lead or other poisonous material is employed, 20 so that it can be used either on damp or wet surfaces without being injuriously affected by the moisture, or in a dry state without the risk of fine particles of its adhesive composition being disseminated in the atmosphere and 25 prejudicially affecting the health of the user.

The present invention therefore consists in a waterproof sheet abrasive material in the preparation of which no lead or other poisonous agent is employed.

30 The process described in the specification of the pending application for patent above referred to consists, as applied to the manufacture of waterproof sandpaper, in running paper forming the base from a reel, from which 35 it passes (after if desired being printed on the back) into a bath of linseed oil which is kept at a temperature of at least 100° C. A small proportion (say about 0.5 per cent) of paraffin or other suitable wax is added to the linseed oil bath, to increase the waterproofing 40 effect.

From this bath the paper preferably passes 45 between a pair of pressure rollers to remove any surplus of the waterproofing material, and which are also kept heated to 100° C. or over.

It may then be rewound into reel form or 50 pass at once direct to a table or series of hot plates or rollers kept at a temperature of 100° C. or over and while passing over this table or 55 series of hot plates or rollers the adhesive employed to secure the abrasive to the paper is applied in any suitable manner. This adhesive, which consists of a mixture of a drying oil (such as linseed oil or tung oil) with a

gum (such as dammar or copal) or synthetic resin, is heated to over 100° C. and applied to the paper while at this temperature.

The following is an example of a suitable composition for this adhesive, viz:

|                     | Parts<br>by weight. |
|---------------------|---------------------|
| Linseed or tung oil | 30                  |
| Dammar or copal gum | 40                  |

In the sequence of operations the paper thus waterproofed and coated with adhesive passes from the table, hot plates or rollers, and the sand (or other abrasive) is applied in any suitable manner. The paper is then baked at 65 a temperature of over 100° C. Subsequently 70 a second or sizing coating of adhesive is applied, according to common practice, after which the sheet abrasive is rebaked (at a temperature of over 100° C.) and the paper will 75 then be ready for use.

The process above described may be modified by the addition, to the adhesive composition above described, of a small proportion (for instance from 2½ to 5 per cent) of paraffin or other suitable wax. In this case the 80 paper, after passing from the table or hot plates or rollers where the adhesive is applied, is next chilled, after which the abrasive is applied. The paper thus coated passes between hot rollers to press the abrasive down into the 85 warmed adhesive composition, after which it is baked at at least 100° C. as before, but the second or sizing coating of adhesive and the subsequent rebaking will not be necessary.

The various baking operations above referred to may be carried out in an oven or other suitable heating apparatus, and it will be found that the operation will be improved 90 in many cases if a current of heated air is caused to pass therethrough by any suitable 95 means.

It will be obvious that by the use of the process above described the employment of volatile thinners in the waterproofing and adhesive materials is obviated, with the 100 avoidance of the risk of fire and danger to workers from the inhalation of the vapors of such volatile thinners.

What we claim and desire to secure by Letters Patent is:

1. A waterproof sheet abrasive material comprising a base, a waterproofing composition applied to such base as a preliminary treatment and consisting of linseed oil with a 110 small proportion of paraffin wax, an adhesive

- composition subsequently applied and consisting of a drying oil with a gum, and an abrasive material.
2. A waterproof sheet abrasive material
- 5 comprising a base, a waterproofing composition applied to such base as a preliminary treatment and consisting of linseed oil with a small proportion of a suitable wax, an adhesive composition subsequently applied and
- 10 consisting of a drying oil with a gum, and an abrasive material.
3. A waterproof sheet abrasive material comprising a base, a waterproofing composition applied to such base as a preliminary
- 15 treatment and consisting of linseed oil with a small proportion of a suitable wax, an adhesive composition subsequently applied and
- 20 consisting of a drying oil with a synthetic resin, and an abrasive material.
4. A waterproof sheet abrasive material comprising a base, a waterproofing composition applied to such base as a preliminary treatment and consisting of linseed oil with a small proportion of paraffin wax, an adhesive composition subsequently applied and
- 25 consisting of a drying oil with a gum and a small proportion of paraffin wax, and an abrasive material.
5. A waterproof sheet abrasive material
- comprising a base, a waterproofing composition applied to such base as a preliminary treatment and consisting of linseed oil with a small proportion of a suitable wax, an adhesive composition subsequently applied and
- 30 consisting of a drying oil with a gum and a small proportion of a suitable wax and an abrasive material, as specified.
6. A waterproof sheet abrasive material comprising a base, a waterproofing composition applied to such base as a preliminary
- 35 treatment and consisting of linseed oil with a small proportion of paraffin wax, an adhesive composition subsequently applied and
- 40 consisting of a drying oil with a synthetic resin and a small proportion of a suitable wax, and an abrasive material.
7. A waterproof sheet abrasive material comprising a base, a waterproofing composition applied to such base as a preliminary
- 45 treatment and consisting of linseed oil with a small proportion of a suitable wax, an adhesive composition subsequently applied and
- 50 consisting of a drying oil with a synthetic resin and a small proportion of a suitable wax, and an abrasive material.
- 55

In witness whereof we affix our signatures.

CARL ADOLPHE KLEIN.

ROBERT SKIRVING BROWN.